

106-88

EXAM

110

Oct. 12, 1948.

J. R. PARSONS

2,451,446

LIGHT-WEIGHT FIBER CONTAINING PRODUCT

Filed Sept. 6, 1943



Inventor:  
Joseph R. Parsons  
By: *Thien, Ober, & Meeklenburg*  
*Attys.*

Patented Oct. 12, 1948

2,451,446

## UNITED STATES PATENT OFFICE

2,451,446

LIGHT-WEIGHT FIBER CONTAINING  
PRODUCT

Joseph R. Parsons, Chicago, Ill., assignor to  
United States Gypsum Company, Chicago, Ill.,  
a corporation of Illinois

Application September 6, 1943, Serial No. 501,429

3 Claims. (Cl. 106—88)

1

The present invention relates to a process for the distribution of considerable quantities of finely divided fibrous material throughout a mass of either dry finely comminuted material, or with a mass of such material which has been wetted with a gauging fluid and then caused to become hardened or set.

One of the primary objects of the present invention concerns itself with the blending of relatively large quantities of fibers with a hardenable material such as a clay, cement, gypsum or the like, for the dual purpose of distributing the said fibers therethrough, and also with a view to producing therefrom very light weight masses which do not exhibit any great tendency to slump either during drying, hardening, or firing.

In other words, the present invention enables the production, from suitable materials, of extremely light weight products, which may be either organic or inorganic, or may consist of a mixture of organic and inorganic materials. Exemplificative of such products are insulating blankets, insulating blocks, and sheets of organic material or of a mixture of organic or inorganic materials, or of finished boards or planks, and insulating sheets, which may or may not be covered externally with cover sheets.

In accordance with the present invention it has been discovered that light weight products may be produced from a mixture of a gaseous emulsion with fiber, either with or without setting or hardening materials, which products will be extremely light in weight and which can be made with a minimum amount of fluid additions.

As a result of the practice of the present invention, the hitherto prolonged and expensive drying of the products is to a large extent obviated, or rendered very much less troublesome, by virtue of the fact that not so much initial moisture has been introduced as by the processes hitherto in use.

The fundamental and essential feature of the present invention resides in the discovery by the inventor that an emulsion, containing gaseous bubbles, may have distributed therethrough, very evenly and uniformly, if desired, a large amount of fibrous or dry material, or both; and that the resulting mixture may be incorporated with large quantities of setting or hardenable materials under such conditions that the fiber-emulsion mixture may become uniformly distributed through the large mass of setting or hardenable material.

More specifically, the invention concerns itself with the manufacture of light weight insulating products made up of either a cementitious ma-

2

terial or a non-setting material such as clay or kaolin, which can be hardened by subsequent firing, and a certain amount of fiber which, prior to the introduction thereof into the gaseous emulsion, has been dried so that the fiber will tend to absorb a considerable quantity of the liquid portions of the emulsion without, however, causing it to break. Consequently, the fibers are kept in a state of loose aggregation, the fiber extending in all three cubical dimensions, thus reinforcing the product and preventing it from slumping or shrinking to any great extent during the drying operations.

For instance, a given amount of gauging fluid or water may have added thereto certain hereinafter more definitely defined surface-tension reducing agents and colloidal material whereafter this gauging fluid or water may be whipped so as to incorporate therewith a large volume of gaseous bubbles with the result that the initial volume of the liquid will be greatly increased, for example, five-fold. That is to say, starting, for instance, with 100 cubic centimeters of the emifiable material in the form of the liquid, this may, by suitable whipping, be converted into 500 cubic centimeters of a gaseous emulsion. It will be self-evident that there will be no increase in weight as a result of such emulsification. There will, however, result a very light weight gauging fluid which can be substituted almost volume for volume for an unemulsified liquid.

Fibrous material may be blended with such an emulsion so that it will tend to become distributed about and between the interfaces of the gaseous bubbles and the liquid, thus becoming oriented in all three cubical dimensions, but held in position by the relative non-collapsibility of the said bubbles. This relative non-collapsibility of the bubbles can be secured by choosing suitable surface-tension reducing agents for the production of the bubbles, and suitable reinforcing colloids to prevent their collapse upon the admixture therewith of the aforementioned water-absorptive fiber. After attaching themselves to the fibers and filler particles, eventually the bubbles break, giving up their water which may be held mechanically in the interstices of the fibers or combined chemically therewith, producing hydrates.

Depending upon the proportions used, various light weight products can be made, among which may be mentioned the following: gypsum board, acoustical tile, acoustical plaster, insulating products, gypsum insulating ties, nailable gypsum boards, nailable cement boards, ceramic insulat-

ing brick, light-weight ceramic products, asphalt insulating products, pipe covering, roof insulation, insulating blankets, insulating tiles, packing materials, and fiber boards.

The relative density of the material is completely under the control of the operator and may be modified by the kind of materials used.

One of the important features of the present invention resides in the broad discovery that a gauging fluid which has been rendered specifically lighter, or has been reduced in density, by the introduction thereinto of gaseous bubbles, will behave, volume for volume, about the same as a plain liquid. In other words, if, for instance, a certain type of calcined gypsum would have a consistency, let us say, of 63 cubic centimeters (which means that 100 grams of the calcined gypsum requires 63 cubic centimeters or grams of water to produce a flowable slurry), this can be converted into a light-weight slurry by the addition of a pregenerated gaseous emulsion weighing approximately 20 grams, or the light-weight slurry made by the conventional method would now have a consistency of 83 cubic centimeters. That is to say, 63 cubic centimeters are used to gauge the calcined gypsum, and 20 cubic centimeters form the foam solution. However, by my method a light-weight slurry which is moldable could be made using a total of 50 cubic centimeters of fluid, if the dry calcined gypsum were added to a light-weight gaseous emulsion; that is to say, actually 30 cubic centimeters less of fluid would be used in my process as compared to the conventional method of producing a light-weight slurry. This is a rather surprising discovery, for ordinarily one would certainly believe that the admixture of so small a quantity by weight of water with so large a quantity of a dry, water-absorbing material such as gypsum, would cause a complete collapse of all of the bubbles in the emulsion, with the production of a dry crumbly mass.

As a matter of fact, however, it appears that in the present case the bubbles act as a sort of a solution lubricant, which enables this relatively small amount, by weight, of water to wet all of the gypsum. Now, if to such an emulsion of gaseous bubbles in water there be first added a relatively large amount of fibrous materials, and these be then mixed with the gypsum, it will be found that the fibers will be carried into all portions of the resulting mixture, becoming very uniformly distributed therethrough. If such a mass is then dried, it will form an extremely light weight product, primarily by the presence of the large amount of fibrous material which will be found in the product distributed in all three cubical dimensions. Thereafter, the fibers will be cemented to each other at all their points of mutual contact, thus preserving the open, porous nature of the resulting product.

The more specific aspect of the present invention will now be described in connection with certain practical examples which are illustrative of the invention, but are not intended to limit the same:

More specifically, as when producing light weight insulating materials, the process involves the production of a stable emulsion of gas bubbles followed by the incorporation with said emulsion of fibrous materials, such as cellulosic or mineral fibers and the like, after which there is added to the mixture thus obtained a hardenable substance, such as cement, calcined gypsum, clay,

synthetic resins, farinaceous products and the like.

Accordingly applicant has devised a number of different types of gaseous emulsions which, for example, may be made from aqueous liquids containing a mucilaginous organic substance and a material which either lowers the surface tension of the aqueous solution or by some other method imparts to it the property of entrapping air bubbles when these are introduced into the mixture, such as by whipping it or by blowing air into it or producing gas bubbles therein by chemical reaction. In any event, the emulsion is first made with a minimum amount of liquid relative to the amount of fibrous material subsequently to be incorporated, whereafter the addition of the fibrous material, such for example as cellulosic or lignous cellulosic fibers, mineral fibers, etc., can be effected. In other words, the fibrous material is added to the emulsion so that the fibers will tend to orient themselves in the interfacial walls of the therein dispersed bubbles, whereafter, by proper mixing, they eventually become substantially uniformly distributed through the emulsion, forming therewith a homogeneous mixture. The fibers absorb some of the liquid of the emulsion thus rendering it thicker and more stable. If one were to allow such a mixture to dry, the fibers would form a very loose state of aggregation which would lack, however, any great degree of cohesion unless the emulsion had contained some adhesive material. For some purposes such a product might be sufficient, particularly where rigidity is not essential. However, in the manufacture of commercial products, where rigidity, or at least a state of adherent aggregation, is desirable, it is necessary to add to the fiber-emulsion mixture some substance which will eventually cement the fibers together at their points of mutual contact so as to lend the necessary rigidity to the product. It will at once be self-evident that the apparent density of such a product may be controlled with considerable accuracy and is, broadly speaking, a function of the amount of heavier setting materials used with respect to the fibrous materials present, and the amount of water used to produce the emulsion. It is sometimes advantageous to vary the viscosity of the gaseous emulsion, depending upon the size and type of fiber or other additive employed. This can be accomplished by blending two or more gas entraining agents or by increasing the concentration of such agents in solution.

Applicant has found that he can produce adherent aggregates of fibrous material which weigh less than one pound per cubic foot and may be varied up to 45 pounds per cubic foot, depending upon the setting materials used and somewhat also upon the nature of the materials from which the emulsion is originally produced and also of course upon the nature and other physical properties of the fibrous material employed.

Generally speaking, applicant's products in their more advantageous commercial aspects are prepared from emulsions consisting of a continuous phase made up of aqueous solutions, or perhaps more accurately speaking, dispersants, of farinaceous materials such as starch, cereal flours and the like, or other gummy or mucilaginous substances, which solutions also contain some surface-tension depressant in the nature of a soap or of one of the many present day available so-called "wetting agents." It has been found that an emulsion consisting of dispersed air bubbles in a solution obtained by boiling starch with water,

and which solution may either contain or have incorporated therewith some wetting agent such as saponin, soap, resin soap, or synthetic organic wetting agent, or a blend of such materials may be readily prepared, thus incorporating a large volume of stable bubbles in the liquid by the process of whipping the latter, very much on the order in which cream or white of eggs are whipped. The effect is of course the entrapment in the fluid of myriads of small air bubbles. In general, the finer the bubbles the more desirable is the emulsion for the purposes of the present invention.

The invention is however not limited to an emulsion prepared by mechanical agitation or whipping, as the bubbles may be incorporated with the liquid by means of forcing streams of air bubbles into the liquid, preferably accompanied by violent agitation or by the expedient of having present in the liquid as initially formed a component of an active mixture, where afterwards a second component is incorporated, which by reaction with the first component will liberate gas bubbles. Examples of such mixtures would be, for instance, a starch solution containing for example saponin or some other wetting agent, and also some sodium bicarbonate, whereafter the liquid may be mixed with aluminum sulfate or with an acid which will react with the bicarbonate through the formation of a salt and the simultaneous development of carbon dioxide bubbles. Other means for creating bubbles would be to have the solution alkaline and to add, for example, metallic aluminum in finely powdered form, or else to develop bubbles in the starch and wetting agent solution by incorporating a gas developing chemical such as calcium carbide and the like. In other words, the method of forming the gas emulsion is of no particular essence and applicant reserves to himself the right to produce the emulsion used in his process by any of the above indicated methods.

The fibers used in connection with the present invention may be of a mineral nature such as mineral wool, glass wool, rock wool, and the like, or they may be organic in nature such as wool, hair, cotton, wood or other forms of cellulose, or mixtures of fibers, either organic or inorganic, or combinations of these. For commercial purposes, however, it has been found that ground wood, and particularly the fibers produced by hammer-mill grinding of old paper such as newspaper and magazines, produces a fibrous aggregate of particular effectiveness in connection with the present invention. It appears that the gas bubbles in the emulsion act as a sort of solution lubricant for the low tensile fiber employed, thus causing the spreading of the fiber individually throughout the entire emulsion structure. Moreover, the emulsion itself contains a relatively large volume of gas as compared with the volume occupied by the water, so that only the surfaces of the fibers are dampened. This prevents any undesired weakening of the fibers, and at the same time produces a much stronger structure than could be obtained were the mixture made by suspending the fibers in the liquid prior to producing the gaseous bubbles therein. At the same time, some of the liquid is abstracted from the foam, thus rendering it stiffer and more stable.

In the present method of operation, no excess of water is used, thus necessitating but a minimum of drying, and allowing the use of a wide variety of fibers. Moreover, the resulting interlaced fiber structure is held intact so that it is not necessary, as has been the case with the prior art,

to use suction to remove the excess water when forming the insulating materials into their desired shape.

The type of wetting agents employed varies very widely and may consist of soap bark, rosin soaps, other organic soaps or synthetic wetting agents, or mixtures of these materials. A great many of these are now available under various trade names, and are very well known in the art. It should be noticed that in the present invention, after the gaseous emulsion has first been prepared, the fibers are added dry, whereafter the setting material is also added in the dry form. The dry addition of the fibers helps to absorb water from the gas emulsion.

As specific examples of the production of various types of insulating materials, the following may be cited:

#### Example I

In this example the object is to prepare a sound-insulating material in the form of acoustical tile. This obviously also will inherently have heat-insulating as well as sound-insulating properties. A dried product weighing about 24 pounds per cubic foot may be prepared by employing about 100 cubic centimeters of a 2% solution of a so-called thin-boiling starch. This solution is prepared by suspending say 20 grams of the raw starch in 1000 cubic centimeters of water, and then bringing this mixture to the gelatinizing point of the starch, which is slightly below the boiling point of the water. To the starch solution thus obtained, which is a fairly fluid liquid, but having a greater viscosity than water, there are added about 15 grams of a wetting agent, for example the one known as DuPont's MP189, which is a well known type of wetting agent consisting essentially of a sulfonated hydrocarbon. The solution thus produced is violently whipped until all of the liquid has been converted into a gas-containing emulsion, and practically no liquid free of bubbles remains. In other words, substantially the entire 1000 cubic centimeters of solution are converted into an emulsion. This will occupy a space from four to five times as great as that of the initial solution. There are then added, separately or in admixture, the following amounts of fibrous material, to-wit, 50 grams of dry ground-wood fiber, and 100 grams of dry sulfite paper pulp ground in a hammer-mill. The incorporation of the emulsion and the fiber is accomplished by means of a commercial mixer which gradually folds the emulsion over and over as the fiber is added so that a thorough incorporation of the fiber and the emulsion is obtained. As an alternative, a commercial mixing machine on the principle of an egg beater, preferably with a revolving tank or bucket, may also be employed. In any event, the 150 grams of fiber are thoroughly incorporated with the emulsion until a substantially uniform mixture is obtained. Thereafter there are gradually sifted into the mixture about 850 grams of calcined gypsum. For this purpose applicant prefers to use that particular type of low consistency gypsum which has become known in the industry under the general designation of "alpha" gypsum, and which is more fully described in the patent to Randel and Dailey No. 1,901,051.

There is also added, preferably in admixture with the "alpha" gypsum, about 15 grams of an accelerator such as terra alba. This terra alba, in the present case, refers to a finely ground natural gypsum, which is calcium sulfate dihydrate.

The setting of the gypsum gives eventual stability to the product being made. However, before the gypsum has a chance to set, the mixture is formed into the desired shapes, such as plates, sheets or blocks, which can be accomplished by pouring the mixture into suitable molds which may be made of wood, metal, rubber, plastics or the like. It is possible under these conditions to produce also various surface characteristics in the finished product and to give it the appearance of artificial stone such for example as travertine. This may be done by providing the face of the mold with irregularly shaped particles of a resilient material such as rubber, hardened water-insoluble gelatin, and the like, or with an ornamental shape. This technique is well known in the stucco molding art. It will be noted that no attempt is made to remove water physically from the mixture. In other words, the 1000 parts of water which have been used to produce the emulsion are absorbed to a considerable extent by the 150 grams of fiber and the 850 grams of the calcined gypsum, so that the entire mass, upon the setting of the gypsum, solidifies into a solid, which is very light in weight, weighing only about 24 to 30 pounds per cubic foot, after drying. After setting has taken place, the product may be liberated from the mold and then allowed to dry either at room temperatures or at slightly elevated temperatures, but in any event at a temperature insufficiently great to re-calcine the formed gypsum dihydrate.

It will be self-evident that coloring matters may be added if desired to give the product a desired shade or tint.

#### Example II

The invention may also be employed for the production of a very light weight wallboard having a gypsum core and covered by two sheets of heavy paper. In itself the manufacture of wallboard is not new, and the present invention therefore relates only to such portion of the making of a gypsum wallboard as involves the preparation of the core material now to be described. This core material, prior to the setting of the gypsum, is placed between two simultaneously advancing sheets of cover paper and allowed to set therebetween. This may be accomplished by means of the well known machines for the manufacture of gypsum wallboard.

In order to illustrate the present phase of the invention, there is submitted herewith a single sheet of drawings in which the figure is a cross section, on a greatly enlarged and exaggerated scale, of gypsum wallboard made in accordance with the present invention.

To prepare the core material one may proceed as follows: 90 grams of a thin-boiling starch are suspended in 1500 cubic centimeters of water and the mixture is heated until the starch has become gelatinized, producing a limpid but slightly viscous solution into which there are then introduced 75 cubic centimeters of a 20% solution of rosin soap in water. The resulting solution is then agitated until its volume has been expanded about four or five times, as a result of the emulsification therewith of countless small air bubbles. After the emulsion has been formed there is incorporated therewith a mixture of 100 grams of dry groundwood and 150 grams of dry sulfite paper pulp which has been hammerfull ground as described in Example I. This fibrous mixture, that is, a total of 250 grams, is thoroughly blended with the emulsion, and thereafter

there is then added thereto 750 grams of ordinary calcined gypsum, that is to say, calcium sulfate hemihydrate, or, as it is also called, commercial stucco. This may contain 25 grams of an accelerator in the form of terra alba, as mentioned in connection with Example I.

After the gypsum and accelerator have been thoroughly incorporated with the emulsion, which may be accomplished in the space of a few seconds, and which is preferably done in the present case just prior to the placing of the core mixture between the fibrous cover sheets 2, the mixture is so placed and the process of making the wallboard continued in the usual fashion. After setting and drying, this will result in a wallboard which, for a thickness of  $\frac{1}{2}$ ", will weigh only about 600 pounds per 1000 square feet. The core 3 containing the fibers and set gypsum is also shown in the drawing.

If the density of this material is calculated on the basis of pounds per cubic foot, it will be found to fall somewhere within the limits between 12 and 20 pounds. As compared with the wallboard cores previously made, this is exceedingly much lighter, as most of the so-called light-weight wallboards have weighed anywhere from 1400 to 1800 pounds per 1000 square feet, even on the  $\frac{3}{8}$ " basis. No wallboard of equivalent light weight has hitherto been proposed or described, and it is one of the outstanding advantages of applicant's invention to prepare such a light-weight wallboard and the like.

#### Example III

In this example a semi-rigid insulating blanket is prepared. This may be folded up or furnished in the form of bats of predetermined dimensions. To prepare such a material one may proceed as follows:

48 grams of a thin-boiling starch are suspended in 60 cubic centimeters of water, and the mixture is heated until the starch has been gelatinized to form a limpid but fairly viscous solution. To this there are then added 12 grams of soap bark, and the mixture stirred until the soap bark has been completely dissolved. The mixture is then beaten until, by the incorporation of a sufficient amount of air bubbles, a total volume of about four to six times the original volume has been obtained.

It will be noticed that in this case the concentration of the primary starch solution is somewhat greater as to its starch content and therefore produces a thicker and even more stable emulsion. To the emulsion thus made there are added 120 grams of dry newspaper which has been disintegrated or ground in a hammermill. At the same time there are also incorporated 50 grams of a commercial asphalt emulsion.

After the starch-gas emulsion, fiber, and the asphalt emulsion have been blended so as to produce a homogeneous mixture, there are then rapidly added 180 grams of calcined gypsum, in this case preferably the "alpha" gypsum already hereinabove fully described. This mixture is then molded into shape, producing for instance bats from  $\frac{1}{2}$ " to 4" in thickness, depending upon the desire of the manufacturer; the mixture so made forming a bat which is sufficiently coherent to permit handling without the necessity of using cover sheets thereon. However, it should be considered as within applicant's invention to cover either one or both sides of these bats with paper cover sheets, and perhaps an impervious asphalted sheet on one side, and a relatively thin and

perforated sheet of paper on the other. The bats thus produced will have a density of as low as 4 pounds per cubic foot, and will not support combustion. They are nevertheless sufficiently self-coherent so as not to shrink or slump in drying. This is the result of the relatively small amount of water used and therefore differentiates the present invention from what has preceded it.

The importance of adding the fibers in dry condition must not be overlooked. Also, the fibers should preferably, but not necessarily, be of a liquid-absorbing nature, so that as much as possible of the liquid portion of the emulsion will be absorbed, or adsorbed, by the fibers. The effect of this is greatly to stiffen the emulsion. The stabilizing film surrounding the individual dispersed air or gas bubbles will, however, not be destroyed, as there will be a certain amount of concentration of the dissolved solids of the emulsion due to the liquid-absorption or adsorption of the fibers. Hence the bubbles will remain as globular aggregates that help to sustain the fibers in their heterogeneous orientation in all three cubical dimensions, which counteracts slumping of the mixture. If a setting substance be present, this, on setting, will then permanently fix the position of all the solid ingredients. As the free liquid disappears, either by combination with the setting substance or by evaporation, or both, the interior space of the bubbles merges with the atmosphere, thus leaving the product highly connectedly porous, as distinguished from unconnected cellularity. Thus while the bubbles form an aggregate during the formation of the mass of material, they ultimately disappear.

#### Example IV

Another type of light weight incombustible insulating blanket or bat may be made as follows:

With 425 grams of water containing 3% of starch, 2% of powdered soap bark and 25 grams of a wax starch suspension, all of which has been agitated until, by the incorporation of finely divided air bubbles, it produces a volume eight to ten times the original volume, I incorporate 35 grams of finely divided cellulose fibers, for instance, kraft fibers, and 165 grams of mineral wool or glass fibers. This aerated fiber mass may then be molded into various shapes of any desired thickness, up to practical limits of better than 8 inches in height, either in separate units or in a continuous ribbon, thus forming a blanket or bat of any desired width.

The material then is dried and may be cut to any size or shape suitable as block, bat or blanket insulation or cushioning material. The product thus produced may be made to have a density as low as one pound per cubic foot and possess inherent characteristics of resiliency and toughness which will permit it to be used and handled for ordinary insulation purposes. While it is desirable for some purposes to incorporate cellulosic fiber, such as kraft or similar fibers, in order to impart toughness to the resilient product, nevertheless, very satisfactory insulating materials may be produced simply by using inorganic fibers, such as mineral wool, glass wool, etc., without the addition of any other fiber.

I also may incorporate other waterproofing agents in the emulsion, which increase the water resistance of the finished product. Stearates, synthetic resins of various types, rubber latex or rubber emulsions, waxes and materials of similar effect may be used.

In the case of clay products as hereinabove

mentioned, only a temporary "set" of the mass occurs, but final hardness is attained by firing at a suitable ceramic-firing temperature. In the latter case, unless incombustible fibers such as mineral wool, asbestos, or high-melting glass wool has been used as the fibrous material, the fibers will be burnt away, thus still further increasing the porosity of the material.

#### Example V

A light-weight insulating blanket, having considerable rigidity, can be prepared in accordance with the following formula:

|                                                                                            | Parts by weight |
|--------------------------------------------------------------------------------------------|-----------------|
| 15 Loose mineral wool                                                                      | 165             |
| Kraft fiber (cellulosic)                                                                   | 35              |
| Soap bark                                                                                  | 8               |
| 20 Binder solution, containing 2% of thick-boiling, and 1% of thin-boiling cooked starches | 425             |
| 16% paraffin suspension                                                                    | 25              |

In producing this material, the soap bark is dispersed in the 425 parts of the binder solution, and the mixture is entirely converted into a gas emulsion weighing about 4 pounds per cubic foot. Thereafter the dry fibers (mineral wool and kraft) are slowly added; whereupon the wax suspension is added and the mixing continued for a short time to insure uniformity. The resulting mixture is then placed into molds and allowed to harden therein, afterwards being dried. If desired, the above material can be colored, for example, a pinkish red, by the incorporation of about 4 parts by weight of iron oxide. The resulting bats may, if desired, be covered with cover sheets of any desired kind.

#### Example VI

Under some circumstances it may be desirable to have a non-uniform distribution of fibers in the mixture. This can be accomplished by using nodulated wool, or so-called "granulated mineral wool," the nodules being added to the gas emulsion. The individual nodules, while they will become distributed in the bubbly mixture, will not lose their internal structure or identity, and hence the product will be non-uniform so far as its texture is concerned. As to relative quantities and mode of operation, Example V is a guide.

#### Example VII

A light weight resilient insulating blanket may be produced from a gaseous emulsion of a soap and rubber, in accordance with the following formula:

|                           |         |     |
|---------------------------|---------|-----|
| Common white (ivory) soap | grams   | 8   |
| Water                     | cu. cm. | 250 |

This mixture is beaten into a gaseous emulsion until most of the free water has disappeared. There are then added

|                                                                                       |       |     |
|---------------------------------------------------------------------------------------|-------|-----|
| Paper pulp (dry)                                                                      | grams | 100 |
| and the pulp uniformly dispersed into the gaseous emulsion; whereupon there are added |       |     |

|                                                                                                                           |       |    |
|---------------------------------------------------------------------------------------------------------------------------|-------|----|
| Rubber emulsion                                                                                                           | grams | 50 |
| and the mixture stirred for a short time to make it homogeneous. It is then molded without filtration and allowed to dry. |       |    |

The rubber emulsion itself contains about 60% of solids consisting of reclaimed rubber dissolved in asphalt and emulsified by means of a small amount of sodium hydroxide. Such emulsions of rubber are well-known articles of commerce.

As the mixture dries, the rubber emulsion breaks and the particles of rubber serve as a cementing agent to affix the paper fibers to each other at their points of contact.

The present invention is of broad applicability, and is only to be limited in scope by the claims appearing below. Obvious modifications of the invention and its applicability to the production of insulating structures of more complicated shape are of course to be considered within the scope of the invention. Furthermore, other cementitious materials such as fast setting cements, as for instance those of the Portland cement type, or the use of other setting materials, such as Sorrel cements, may be employed. In fact, any inorganic substance which will readily mix with the water present is to be considered as encompassed within the purview of the invention. Moreover, the use of other dryable adhesive materials such as cellulose ethers (for example, methyl cellulose), polyvinyl alcohol, casein, vegetable protein, glues, water-soluble gums such as gum arabic, tragacanth, etc., are also to be considered as within the scope of the invention.

From the foregoing examples it will be self-evident that a broad invention has been disclosed. However, in order to preserve a line of division between heavy products and light products, applicant has claimed the production of relatively heavy products, such as are devoid of fiber, in his co-pending application, Serial No. 501,428, filed of even date herewith.

Applicant claims:

1. Process of producing semi-rigid insulating bats which comprises preparing a solution of a farinaceous material and a surface-tension reducing agent in water, incorporating a large number of small discrete air bubbles with said solution to form an emulsion of gas and water, incorporating dry water-insoluble fibers with the emulsion thus produced, thereupon blending the resulting mixture with an asphalt emulsion and with dry calcined gypsum, forming the final mixture thus produced into the desired shape without the application of substantial pressure thereto, and drying the thus shaped product. 45

2. Process of producing light-weight porous insulating material which comprises whipping an

aqueous starch solution containing a surface tension depressant into a stiff gaseous emulsion, stirring dry water-absorbent fibers into said emulsion, and distributing them therein, thereupon adding and thoroughly admixing dry powdered calcined gypsum with the thus prepared fibered emulsion, forming the resulting mixture into a predetermined shape, causing it to set up as the result of the hydration of said calcined gypsum, and drying the product thus obtained.

3. Process of producing light-weight porous insulating material which comprises the steps of preparing a solution of a water-soluble colloidal organic bonding agent and a surface tension reducing agent in water, incorporating with said solution a large number of small individual bubbles so as to form an emulsion, incorporating dry water-insoluble fibers with the emulsion thus produced, and then adding dry calcined gypsum to the resulting mixture and shaping the final mixture into shape substantially without the application of pressure thereto, permitting said gypsum to set, and eventually removing any residual water by evaporation thereof.

JOSEPH R. PARSONS.

REFERENCES CITED

The following references are of record in the file of this patent:

UNITED STATES PATENTS

| Number    | Name          | Date          |
|-----------|---------------|---------------|
| 1,613,137 | Seigle        | Jan. 4, 1927  |
| 1,742,794 | Storey et al. | Jan. 7, 1930  |
| 1,880,601 | Untiedt       | Oct. 4, 1932  |
| 1,901,057 | Roos          | Mar. 14, 1933 |
| 1,944,008 | Hobart        | Jan. 16, 1934 |
| 2,007,133 | Roos          | July 2, 1935  |
| 2,023,800 | Williamson    | Dec. 10, 1935 |
| 2,053,842 | Rice          | Sept. 8, 1936 |
| 2,292,012 | Parsons       | Aug. 4, 1942  |
| 2,322,194 | King          | June 15, 1943 |

FOREIGN PATENTS

| Number  | Country       | Date |
|---------|---------------|------|
| 487,259 | Great Britain | 1938 |
| 531,469 | Great Britain | 1941 |